

## 1

3,002,616

**POTASH ORE BENEFICIATION PROCESS**  
 John H. Sholine, Lakeland, Fla., and Charles C. Cook,  
 Aiken, S.C., assignors to International Minerals &  
 Chemical Corporation, a corporation of New York  
 No Drawing. Filed Mar. 5, 1958, Ser. No. 719,203  
 8 Claims. (Cl. 209—2)

The present invention relates generally to a process for beneficiating ores and particularly to a process for beneficiating potash ores. More particularly the present invention relates to a process for beneficiating potash salts comprising langbeinite, sylvite and halite using an air tabling operation.

As is well known, potash is of great economic importance. The sources of potash are very numerous. Extensive deposits of potash salts are found on every continent. However, in practically no instance is the potash salt found as a substantially pure salt. On the North American continent, one frequently encountered potash salt is sylvite (KCl). The KCl is not often found in any appreciable quantities as pure sylvite ore but is most often found as the sylvite ore, which is a mixture of KCl and NaCl. Sylvite ores sometimes have a high purity of approximately 96%, and a typical analysis of such an ore is as follows:

|                                                                               | Percent |
|-------------------------------------------------------------------------------|---------|
| Sylvite (KCl)-----                                                            | 31      |
| Halite (NaCl)-----                                                            | 65      |
| Other constituents or impurities consisting of silicates, sulfates, etc.----- | 4       |

The sylvite values of ores of such a high purity may readily be recovered or concentrated by various concentration processes, such as crystallization, electrostatic separation, flotation separation, etc. As the natural deposits of ores of such high purity are depleted, it has been necessary to resort to ores of less purity. In some instances, however, it has been found that the impurity in the ore is troublesome in the concentration process. Langbeinite ( $K_2SO_4 \cdot 2MgSO_4$ ) is a commonly occurring impurity in sylvite ores and at relatively high concentrations of langbeinite it is often difficult to separate or concentrate the sylvite values in the potash ore.

A typical analysis of such an ore is as follows:

|                                              | Percent |
|----------------------------------------------|---------|
| Sylvite (KCl)-----                           | 10.6    |
| Halite (NaCl)-----                           | 53.2    |
| Langbeinite ( $K_2SO_4 \cdot 2MgSO_4$ )----- | 33.9    |
| Other constituents or impurities-----        | 2.3     |

Accordingly, it is an object of the present invention to provide a process for beneficiating a potash ore containing langbeinite.

It is another object of the present invention to provide a process for beneficiating a potash ore containing langbeinite to obtain a concentrate of increased potash concentration and decreased langbeinite concentration.

A further object of the present invention is to provide a process for beneficiating a sylvite-halite ore containing langbeinite in an amount greater than 7% by weight, to obtain a concentrate containing sylvite in an increased concentration and langbeinite in an amount less than 7% by weight.

These and other objects and advantages of the present invention will be apparent to those skilled in the art as the description of the present invention progresses.

In accordance with the present invention, it has been discovered that eminently satisfactory dry beneficiation of ores and minerals can be achieved through air tabling by means of a series of critical and interdependent process steps. Generally described, a potash ore containing langbeinite is first comminuted to substantially liberate

## 2

the particles of the ore. The comminuted ore is then subjected to an air tabling operation, whereby a concentrate is obtained which has a higher potash concentration and a lower langbeinite concentration than the original ore. This concentrate is then sized to produce a fraction whose average particle size is larger than the average particle size of the concentrate. It has been found that this larger size fraction has a higher potash concentration and a lower langbeinite concentration than the concentrate recovered from the tabling operation.

In this novel process, potash ore containing langbeinite, for example sylvite ore containing langbeinite as received from the mine, is comminuted to economical liberation size to produce a granular feed material. The comminution of the ore to the liberation of the various constituents to be separated is effected to liberate a substantial amount of the various constituents. It may be desirable or economical to comminute the ore to liberate all of the constituents, however, the ore may be liberated to a lesser extent, for example to 70-80% liberation. This granular material is sized to produce a granular feed of a particle size in the range of about -8 mesh and preferably a feed consisting of -8+200 mesh particles and still more preferably a feed consisting of -8+150 mesh particles. The comminution of the ore may be carried out in a ball mill, roller mill, hammer mill, or any other suitable type of grinding or crushing apparatus. When the ore is ground to the mesh size indicated above, the sylvite values, the halite values and the langbeinite values are substantially separated from each other and the ore is ready for further treatment in accordance with this invention.

After the comminution step of the process the ore may be passed directly to the air tabling zone or it may be sized before the air tabling operation. It is frequently desirable to size the ore prior to the air tabling operation since a sized feed in an air tabling operation results in a greater screen load or sizing load and a smaller table load.

The screened ore is then passed to an air tabling zone wherein the ore is subjected to an air tabling operation. A sylvite concentrate is separately recovered from the air tabling zone and a langbeinite concentrate is also separately recovered from the air tabling zone. While the operation is herein described as producing only two fractions or concentrates, it is to be understood that other fractions may also be produced in the air tabling zone. For example, a so-called mids fraction is usually produced and is most often recycled to the tabling zone in admixture with the fresh feed.

In the air tabling zone the comminuted potash ore is subjected to an air tabling operation. An air table is a shaking table in which air blown through a porous deck, which is preferably riffled, coats with the shaking to fluidize a layer of dry solids moved lengthwise of the deck by a quick-return shake. The deck of the apparatus is canted somewhat on the longitudinal center line. The granular friction of the lighter gravity particles is overcome by the continual impingement of low-pressure air on the lower surface of the particles, thereby giving them fluidity, the velocity of the air being maintained to a degree that only the lighter gravity particles are affected. The semi-fluid mass formed on the deck stratifies and moves lengthwise on the deck due to the quick-return shaking action and moves downslope on the canted deck under the influence of gravity. The concentrates and other fractions are removed at the edge of the deck. Air tabling apparatus of this type is well known. Examples of commercially available air tables are the Sutton-Steel table, known as the "airfloat" or Kupp-Kelly table, the Birtley table, and the Knapp and Bates (K and B)

table. Air jigs or tables similar to the Roberts and Schaefer airflow coal cleaner are also effective.

Factors to be considered in an air tabling operation are: the extent of the spread of air as it leaves the deck and impinges upon the mineral particle, the velocity of the air impinging on the particles, the size of the particles, the range of particle sizes, and the shape of the particles.

The langbeinite ore particles have a specific gravity of from about 2.6 to about 3.1 and are relatively heavier than the sylvite and halite ore particles, which have a specific gravity of from about 1.7 to about 2.3. A langbeinite concentrate and a sylvite concentrate are, therefore, separately recovered in the air tabling operation.

The langbeinite concentrate obtained from the air tabling operation, when compared with the ore charged to the tabling zone, has a substantially higher langbeinite concentration and a substantially lower sylvite concentration. The langbeinite concentrate may be recovered as a product or may be additionally concentrated in a further concentrating operation.

Similarly, the sylvite concentrate obtained from the air tabling operation, when compared with the ore charged to the tabling zone, has a substantially higher sylvite concentration and a substantially lower langbeinite concentration. It has been found that when the sylvite concentrate is sized to produce a larger sized fraction, that is, a fraction whose average particle size is larger than the average particle size of the concentrate, that the larger sized fraction has a still higher sylvite concentration and still lower langbeinite concentration. Therefore, in accordance with the present invention, the sylvite concentrate is subjected to a sizing operation. Any suitable type of sizing such as sedimentation, elutriation, screening, etc. may be used and a screening operation has proven to be very satisfactory. It has been found preferable to size the sylvite concentrate so as to produce a substantially +50 mesh size fraction and a substantially -50 mesh size fraction. A sizing around the 50 mesh size is preferred since the +50 mesh size fraction has been found to be very high in sylvite concentration and relatively low in langbeinite concentration. A separation around a mesh size different than 50 may be used; however, the sizing will preferably be done about a mesh size within the range of from about 20 mesh to 80 mesh, that is, the small size limit for the larger size fraction will be within the range of from about 20 mesh to about 80 mesh. It is also within the scope of this invention to size the sylvite concentrate from the air tabling zone so as to produce more than two sized fractions.

It has further been found that the smaller sized fraction recovered from the above screening operation may have the constituents substantially separated when it is subjected to another air tabling operation. The air tabling operation on the smaller sized fraction is generally similar to the air tabling of the original potash ore. The average size of the particle is, however, smaller because of the sizing operation. Accordingly, it may be necessary to decrease the flow rate of air through the deck of the table and make other adjustments so as to obtain optimum separation of the components of the ore. A langbeinite concentrate and a sylvite concentrate are separately recovered from the air tabling operation on the smaller sized particles.

The langbeinite concentrate obtained from this latter air tabling operation, when compared with the smaller sized fraction charged, has a substantially higher langbeinite concentration and a substantially lower sylvite concentration. This langbeinite concentrate may be mixed with the langbeinite concentrate obtained in the first tabling operation. Similarly, the sylvite concentrate obtained from the air tabling of the smaller sized fraction, when compared with the charge to this air tabling zone, has a substantially higher sylvite concen-

tration and a substantially lower langbeinite concentration. This sylvite concentrate may be combined with the larger screen size sylvite concentrate obtained from the screening operation to give a final sylvite concentrate of the process.

The langbeinite concentrates and the sylvite concentrates obtained according to the process of this invention may be further concentrated if desired or they may be separately recovered as products of the process.

In order to give a fuller understanding of the invention, but with no intention to be limited thereto, the following specific example is given.

#### Example

Natural sylvinitic ore from the Carlsbad section of New Mexico was comminuted in a roll crusher and then in the hammer mill. The comminuted ore was screened to produce a -8 mesh fraction. Substantially all of the fraction contained particles in the range of -8 mesh to about 200 mesh size. The fraction had the following analysis:

|                        | Percent |
|------------------------|---------|
| Langbeinite            | 33.89   |
| KCl                    | 10.61   |
| Remainder, mostly NaCl | 55.50   |

This fraction was subjected to a tabling operation using a Sutton and Steele model V-80 air table. A sylvite concentrate and a langbeinite concentrate were separately recovered. The sylvite concentrate was 40.4% by weight of the original charge and the langbeinite concentrate was 59.6% by weight. The analyses of these fractions were as follows:

|                             | Percent |
|-----------------------------|---------|
| 35 Sylvite concentrate:     |         |
| Langbeinite                 | 12.5    |
| KCl                         | 18.0    |
| 25 Langbeinite concentrate: |         |
| Langbeinite                 | 48.4    |
| KCl                         | 5.5     |

The sylvite concentrate was then sized at 50 mesh (Tyler screen size) and a +50 mesh fraction and a -50 mesh fraction were separately recovered. The -50 mesh fraction was 19.9 weight percent of the original sylvinitic or charged to the tabling operation and the +50 mesh fraction was 20.5%. The analyses of these fractions were as follows:

|              | Percent |
|--------------|---------|
| 50 -50 mesh: |         |
| Langbeinite  | 15.7    |
| KCl          | 16.4    |
| 50 +50 mesh: |         |
| Langbeinite  | 5.1     |
| KCl          | 21.6    |

It may be noted that the +50 mesh fraction is higher in KCl concentration than the sylvite concentrate obtained from the air tabling operation.

The -50 mesh fraction was then air tabled on the same air table originally used and a sylvite concentrate and a langbeinite concentrate were separately recovered. The sylvite concentrate recovered from this second tabling operation was 15.3% by weight of the original sylvinitic ore fed to the first tabling operation and the langbeinite concentrate recovered from this second tabling operation was 4.6% by weight. The analyses of these concentrates were as follows:

|                             | Percent |
|-----------------------------|---------|
| 60 Sylvite concentrate:     |         |
| Langbeinite                 | 9.0     |
| KCl                         | 16.8    |
| 65 Langbeinite concentrate: |         |
| Langbeinite                 | 39.2    |
| KCl                         | 6.2     |

This sylvite concentrate was combined with the +50 mesh fraction obtained from the screening operation and this combined sylvite concentrate represented 35.8% by

weight of the original ore charged to the process and had the following analysis:

|             | Percent |
|-------------|---------|
| Langbeinite | 6.7     |
| KCl         | 19.0    |

Similarly, the langbeinite concentrate obtained from the second tabling operation was combined with the langbeinite concentrate obtained from the first tabling operation, and this combined langbeinite concentrate represented 64.2% by weight of the original ore charged to the process and had the following analysis:

|             | Percent |
|-------------|---------|
| Langbeinite | 48.7    |
| KCl         | 5.7     |

This example illustrates that following the procedure of this invention a sylvite concentrate containing less than 7% by weight of langbeinite may be prepared from a sylvinitic ore containing more than 7% and as much as 30% by weight of langbeinite.

The description of the invention utilized specific reference to certain process details; however, it is to be understood that such details are illustrative only and not by way of limitation. Various modifications and equivalents of the invention will be apparent to those skilled in the art from the foregoing description.

Having now fully described and illustrated the invention, what is desired to be secured and claimed by Letters Patent is set forth in the appended claims:

1. A process for beneficiating a potash ore containing sylvite, langbeinite and halite constituents which comprises comminuting the ore to the liberation of the various constituents, subjecting the comminuted ore to an air tabling operation and recovering a sylvite concentrate, and sizing said concentrate and recovering a large size fraction of increased sylvite concentration from the sizing operation.

2. A process for beneficiating a potash ore containing sylvite, halite and langbeinite constituents, the langbeinite concentration being greater than 7% by weight, which comprises comminuting the ore to the liberation of the various constituents, subjecting the comminuted ore to an air tabling operation and recovering a sylvite concentrate, sizing said concentrate and recovering a large size fraction having increased sylvite concentration and having a langbeinite concentration of less than 7% by weight from the sizing operation.

3. A process for beneficiating a potash ore containing sylvite, halite and langbeinite constituents which comprises comminuting the ore to produce a -8 mesh fraction, subjecting the -8 mesh fraction to an air tabling operation and recovering a sylvite concentrate, sizing said concentrate and recovering a larger sized fraction of increased sylvite concentration having the smaller size limit within the range of from about 20 mesh to about 80 mesh.

4. A process for beneficiating a potash ore containing sylvite, halite and langbeinite constituents, the langbeinite concentration being greater than 7% by weight, which comprises comminuting the ore to produce a -8 mesh fraction to liberate the various constituents of said ore, subjecting said -8 mesh fraction to an air tabling operation and recovering a sylvite concentrate, sizing said concentrate and recovering a larger sized fraction having the smaller size limit within the range of from about 20 mesh to about 80 mesh, having increased sylvite concentration and having a langbeinite concentration of less than 7% by weight.

5. A process for beneficiating a potash ore containing sylvite, langbeinite and halite constituents which comprises comminuting the ore to the liberation of the various constituents, subjecting the comminuted ore to an air tabling operation and recovering a sylvite concentrate, sizing said concentrate and recovering a large size fraction of increased potash concentration and a smaller size fraction from the sizing operation, air tabling said smaller size fraction and separately recovering a fraction of increased sylvite concentration and a fraction of increased langbeinite concentration.

6. A process for beneficiating a potash ore containing sylvite, halite and langbeinite constituents, the langbeinite concentration being greater than 7% by weight, which comprises comminuting the ore to the liberation of the various constituents, subjecting the comminuted ore to an air tabling operation and recovering a sylvite concentrate, sizing said concentrate and recovering a large size fraction having increased sylvite concentration and having a langbeinite concentration of less than 7% by weight and a smaller size fraction from the sizing operation, air tabling said smaller size fraction and separately recovering a fraction of increased sylvite concentration and a fraction of increased langbeinite concentration.

7. A process for beneficiating a potash ore containing sylvite, halite and langbeinite constituents which comprises comminuting the ore to produce a -8 mesh fraction, subjecting the -8 mesh fraction to an air tabling operation and recovering a sylvite concentrate, sizing said concentrate and separately recovering a larger sized fraction of increased sylvite concentration having the smaller size limit within the range of from about 20 mesh to about 80 mesh and a smaller size fraction, air tabling said smaller size fraction and separately recovering a fraction of increased sylvite concentration and a fraction of increased langbeinite concentration.

8. A process for beneficiating a potash ore containing sylvite, halite and langbeinite constituents, the langbeinite concentration being greater than 7% by weight, which comprises comminuting the ore to produce a -8 mesh fraction to liberate the various constituents of said ore, subjecting said -8 mesh fraction to an air tabling operation and recovering a sylvite concentrate, sizing said concentrate and separately recovering a larger sized fraction having the smaller size limit within the range of from about 20 mesh to about 80 mesh having increased sylvite concentration and having a langbeinite concentration of less than 7% by weight and a smaller sized fraction, air tabling the smaller size fraction and separately recovering a fraction of increased sylvite concentration and a fraction of increased langbeinite concentration.

#### References Cited in the file of this patent

#### UNITED STATES PATENTS

|           |               |                |
|-----------|---------------|----------------|
| 1,939,119 | Holt et al.   | Dec. 12, 1933  |
| 2,175,484 | Rees et al.   | Oct. 10, 1939  |
| 2,307,064 | Patterson     | Jan. 5, 1943   |
| 2,330,479 | Erickson      | Sept. 28, 1943 |
| 2,347,215 | Pattee        | Apr. 25, 1944  |
| 2,487,845 | Bird          | Nov. 15, 1949  |
| 2,745,547 | Werge         | May 15, 1956   |
| 2,849,113 | Bourne et al. | Aug. 26, 1958  |

65

#### OTHER REFERENCES

Taggart: "Handbook of Mineral Dressing," 1945, sec. 11, pages 70 and 73.